

## 1

3,296,019

**POLY(ETHYLENE OXIDE) ADDUCTS OF FATTY OILS AND FATTY AMINES AS ANTISTATIC COATING FOR POLYOLEFIN FIBERS**

Ann S. Keller, Norristown, and Harry H. Hall, Springfield, Pa., assignors, by mesne assignments, to FMC Corporation, San Jose, Calif., a corporation of Delaware

No Drawing. Filed Apr. 19, 1962, Ser. No. 188,838

4 Claims. (Cl. 117—138.8)

This invention relates to finished polyolefin fibers. More particularly, it relates to polyolefin yarns or fibers having applied finishes which enable the yarns to be satisfactorily processed and utilized in the commercial production of textiles and in machine sewing operations.

Polyolefin yarns, for example polypropylene and polyethylene yarns, tend to develop high electrostatic charges and excessive tensions when running over guides, godets and other objects during processing and subsequent handling. The utilization of unfinished polyolefin yarns in textile production and sewing equipment is unsatisfactory.

Static and tension problems have been encountered in the use of other natural and synthetic polymer yarns, and finishes which are satisfactory from both the standpoints of application and use have been developed for them. However, the polyolefins have different physical characteristics than most other filament forming polymers and conventional finishes and methods for application thereof are not suitable or effective in providing the necessary fiber to fiber lubrication, proper fiber to metal frictional behavior, and adequate static suppression.

The primary object of this invention is to provide a finished polyolefin yarn which is suitable for high speed processing, textile and sewing operations.

It is another object of this invention to provide a method of finishing polyolefin fibers which is effective in providing fiber lubrication and static suppression.

These and other objects are accomplished in accordance with this invention with a finish composition for polyolefin fibers comprising from about 10 to about 30% by weight of a finish consisting essentially of 1 to 5 parts by weight of a polyethylene oxide modified fatty oil and 1 part by weight of a polyethylene oxide modified C<sub>12</sub>—C<sub>18</sub> fatty acid primary amine, and from about 90 to 70% by weight of water. This finish composition is applied to polyolefin yarns including, for example, polyethylene, polypropylene and polyisobutylene yarns or fibers by any known means including bath, spray, padding, kiss roll application or the like.

Generally speaking, water base finish compositions are unsatisfactory for application to polyolefin yarn or fibers because of the hydrophobic nature of these polymers. The present finish composition, however, is an exception and provides unexpectedly good lubrication and static suppression.

The fatty oils of the invention include, for example, castor oil, cotton seed oil, flax seed oil, olive oil, peanut

## 2

oil, corn oil, coconut oil, soya bean oil, palm oil, perilla oil, tallow, whale oil, bone oil, etc. If desired, these oils may be partially hydrogenated to increase saturation and vary the melting range thereof.

5 The fatty oils are reacted with ethylene oxide to obtain polyethylene oxide adducts of the fatty oil. The adducts generally have an average or from about 15 to 40 or more ethylene oxide units per glycerine molecule in the fatty oil and preferably from 20 to about 30 ethylene oxide units per molecule.

The fatty acid primary amines of this invention are preferably derived from the amination of fatty acids or a mixture of fatty acids obtained from the distillation of 15 the products of hydrolysis of the above described fatty oils. The C<sub>12</sub>—C<sub>18</sub> fatty acids include, for example, lauric acid, myristic acid, palmitic acid, stearic acid, oleic acid, linoleic acid, etc. Mixtures of these acids, for example 20 those obtained from tallow oil, namely, stearic, palmitic and oleic, are as good or better than individual fatty acids for the purposes of this invention. The fatty acid primary amines are reacted with ethylene oxide to obtain polyethylene oxide adducts of the fatty acid amines wherein 25 each fatty amine molecule has attached thereto a chain having an average of from about 10 to 30 and more ethylene oxide units and preferably from about 15 to 25 ethylene oxide units per molecule of fatty amine.

30 Many lubricant-antistat combinations were investigated to develop a satisfactory finish composition for polyolefin fiber. Before combinations of lubricants and antistats were tried, however, a screening test was conducted to determine whether the lubricant or antistat material would 35 degrade the polyolefin. Screening involved placing approximately 0.2 ml. of the liquid lubricant or antistat onto a sheet of polypropylene film which has been secured to a glass plate. A piece of graph paper was placed 40 between the film and the glass and served two purposes; it would indicate penetration of the film by the liquid, and also give an indication of the spreading action of the lubricant or antistat. The material passed the screening 45 test if 24 hours of film contact produced no change in film appearance such as waviness or puckering. If puckering did occur it was assumed that it was caused by penetration of the lubricant or antistat into the film and this type of behavior would also occur with a polypropylene fiber. Puckering was considered to be caused by 50 plasticization or a similar phenomenon and test materials causing it were rejected.

The above screening test indicated that paraffinic oils and low molecular weight esters had a noticeable undesirable effect on the test film. Applications of these materials to polyolefin yarn at spinning and the consequential softening or plasticization of this yarn corroborated the screening test results.

60 To demonstrate the specificity of this invention there is set forth in the following table a list of finishes, the components of which have passed screening tests but which have been found unsatisfactory either in their application or in their ability to improve characteristics of the yarn.

TABLE I

| No. | Finish Composition                                    | Percent By Weight |
|-----|-------------------------------------------------------|-------------------|
| 1   | Diethyl cyclohexylamine salt of lauryl sulfate        | 3-5               |
|     | Coconut oil                                           | 95-97             |
| 2   | Diethyl cyclohexylamine salt of lauryl sulfate        | 3-10              |
|     | Sorbitan monooleate                                   | 1.5-5             |
|     | Butyl stearate                                        | 85-95.5           |
| 3   | Diethanolamine salt of dilauryl phosphate             | 3                 |
|     | Sorbitan monooleate                                   | 4                 |
|     | Butyl stearate                                        | 93                |
| 4   | 1-hydroxyethyl-2-oleyl ethyl glyoxolinium ethosulfate | 3                 |
|     | Sorbitan monooleate                                   | 3                 |
|     | Butyl stearate                                        | 94                |
| 5   | Sorbitan monooleate                                   | 5                 |
|     | Butyl stearate                                        | 95                |
| 6   | 1-hydroxyethyl-2-oleyl ethyl glyoxolinium ethosulfate | 3                 |
|     | Sorbitan monooleate                                   | 4                 |
|     | Coconut oil                                           | 93                |
| 7   | 1-hydroxyethyl-2-oleyl ethyl glyoxolinium ethosulfate | 5                 |
|     | Sorbitan trioleate                                    | 20                |
|     | Esterified pentaerythritol                            | 75                |
| 8   | Diethyl cyclohexylamine salt of lauryl sulfate        | 10                |
|     | Water                                                 | 90                |
| 9   | Diethyl cyclohexylamine salt of lauryl sulfate        | 10                |
|     | Diethylene glycol                                     | 90                |
| 10  | Diethyl cyclohexylamine salt of lauryl sulfate        | 5                 |
|     | Polyethylene glycol (M.W. 400) monooleate             | 95                |
| 11  | Diethyl cyclohexylamine salt of lauryl sulfate        | 5                 |
|     | Dialiphatic ether of polyethylene glycol              | 95                |
| 12  | Esterified pentaerythritol                            | 60                |
|     | Nonionic emulsifying agents                           | 40                |
| 13  | Finish No. 12                                         | 10                |
|     | Water                                                 | 90                |
| 14  | Finish No. 12                                         | 95                |
|     | Sorbitan monooleate                                   | 3                 |
|     | N-cetyl N-ethyl morpholinium ethosulfate              | 2                 |
| 15  | Finish No. 14                                         | 20                |
|     | Water                                                 | 80                |
| 16  | N-cetyl N-ethyl morpholinium ethosulfate              | 5                 |
|     | Technical grade octanol                               | 95                |
| 17  | N-cetyl N-ethyl morpholinium ethosulfate              | 10                |
|     | Water                                                 | 90                |
| 18  | N-cetyl N-ethyl morpholinium ethosulfate              | 10                |
|     | Diethylene glycol                                     | 90                |
| 19  | N-cetyl N-ethyl morpholinium ethosulfate              | 2                 |
|     | Finish No. 12                                         | 98                |
| 20  | Polyoxyethylene modified tallow acid primary amine    | 5                 |
|     | Polyethylene glycol (M.W. 200) monolaurate            | 95                |
| 21  | Polyethylene glycol (M.W. 200) monopalargonate        | 100               |
| 22  | Polyethylene glycol (M.W. 1000) monostearate          | 2                 |
|     | Polyethylene glycol (M.W. 200) monopalargonate        | 98                |
| 23  | Diethanolamine salt of dilauryl phosphate             | 5                 |
|     | Finish No. 22                                         | 95                |
| 24  | Diethanolamine salt of dilauryl phosphate             | 10                |
|     | Polyethylene glycol (M.W. 200) monopalargonate        | 90                |
| 25  | Polyethylene glycol (M.W. 400) monopalmitate          | 2                 |
|     | Water                                                 | 98                |
| 26  | Diethanolamine salt of dilauryl phosphate             | 10                |
|     | Polyethylene glycol (M.W. 200) monolaurate            | 90                |

In addition to the above yarn finish compositions, many other unsatisfactory combinations were tested which were identifiable only under chemical trade names and/or broad chemical terms.

Polyolefin fibers and in particular polypropylene fibers are much more difficult to finish than other synthetic or natural polymer fibers. They are non-polar materials and as such have no affinity for the usual yarn finishes. They are hydrophobic, and in general, water base finish compositions cannot be used to obtain a satisfactory finish. The polyolefin fibers are degraded by treatment with hydrocarbon oil base compositions and become undesirably soft. For these reasons, the finish composition is extremely critical in order to obtain satisfactory yarn characteristics.

The following examples are set forth to demonstrate finish application and composition in accordance with the invention.

#### Example I

A mixed composition of 2 parts of the polyethylene oxide adduct of hydrogenated castor oil having an average of 25 ethylene oxide units per glyceride molecule of the castor oil and 1 part of the polyethylene oxide adduct of primary amines prepared from fatty acids derived from tallow oil having an average of 20 ethylene oxide units per molecule of fatty amine, was mixed with water at a concentration of 20% by weight. Then, the finished solution was applied to polypropylene ap-

proximately 800 denier, 34 filament yarn by means of a kiss roll 6 inches in diameter and 1½ inches wide just prior to primary take-up. The finished yarn was collected onto a standard take-up tube with ease. The finish was also found to be an aid in processing the yarn through a draw-twisting unit.

#### Example II

A finish was prepared and applied to polypropylene fiber as described in Example I except that 4 parts of the polyethylene oxide adduct of hydrogenated castor oil were used instead of 2 parts and the combination was mixed with water at a concentration of 15% by weight. The fiber was found to have even better processing properties than the finished yarn of Example I.

Various changes and modifications may be made in practicing the invention without departing from the spirit and scope thereof and, therefore, the invention is not to be limited except as defined in the appended claims.

We claim:

- Polyolefin fibers having incorporated thereon a finish consisting essentially of 1 to 5 parts by weight of a polyethylene oxide modified fatty oil having an average of at least 15 ethylene oxide units per glyceride molecule and 1 part by weight of a polyethylene oxide modified primary amine having an average of at least 10 ethylene oxide units per amine molecule said primary amine obtained from a  $C_{12}-C_{18}$  fatty acid.

2. The polyolefin fibers of claim 1 wherein the fatty oil is hydrogenated castor oil.

3. The polyolefin fibers of claim 1 wherein the C<sub>12</sub>—C<sub>18</sub> fatty acid is a mixture of acids derived from tallow.

4. Polypropylene fibers having incorporated thereon a finish consisting essentially of 1 to 5 parts by weight of a polyethylene oxide modified hydrogenated castor oil having an average of at least 15 ethylene oxide units per glyceride molecule and 1 part by weight of a polyethylene oxide modified primary amine having an average of at least 10 ethylene oxide units per amine molecule and wherein said primary amine is obtained from the fatty acids derived from tallow.

**References Cited by the Examiner**

UNITED STATES PATENTS

|           |         |                        |           |
|-----------|---------|------------------------|-----------|
| 1,970,578 | 8/1934  | Schoeller et al. ----- | 260—8.9   |
| 2,614,289 | 10/1952 | Cresswell et al.       |           |
| 2,832,697 | 4/1958  | Walles.                |           |
| 2,999,827 | 9/1961  | McGary et al. -----    | 260—23    |
| 3,009,830 | 11/1961 | Levine -----           | 117—139.5 |
| 3,048,539 | 8/1962  | Kocay et al. -----     | 252—8.8   |
| 3,049,504 | 8/1962  | Swern et al. -----     | 260—23    |

LEON J. BERCOVITZ, *Primary Examiner.*

R. W. GRIFFIN, C. W. IVY, *Assistant Examiners.*